

## UNITED STATES PATENT OFFICE.

BRUCE WINFRED GONSER, OF WOODBRIDGE, NEW JERSEY, AND CALVIN W. HAFFEY, OF SELBY, CALIFORNIA, ASSIGNEES TO AMERICAN SMELTING AND REFINING COMPANY, OF NEW YORK, N. Y., A CORPORATION OF NEW JERSEY.

## LEAD REFINING.

No Drawing.

Application filed February 15, 1928. Serial No. 254,606.

This invention relates to the separation of antimony and tin from lead bullion, and more particularly to a new and improved method for concentrating the tin skim which is produced by heating lead bullion and for removing substantially the entire antimony content from the bullion as a fume.

When lead bullion containing tin, antimony and various other impurities, is heated to a sufficient temperature, the tin becomes oxidized and forms a skim on the surface thereof which must be removed prior to treatment for the elimination of antimony. This skim may contain portions of lead and antimony which must be separated therefrom by subsequent treatment.

When further heat is applied after the tin skim is removed the antimony is oxidized and a portion thereof passes off in the form of a fume, whereas various other portions form a stable oxide which remains upon the surface of the bath as an antimony oxide skim which must be removed from the bath and further treated for the separation of lead.

This invention relates particularly to the concentration of the tin in the tin skim formed in treating the lead bullion and the elimination of lead and antimony and various other substances therefrom. The invention also provides for the elimination of substantially the entire antimony content in the form of a fume with the formation of only a comparatively small amount of antimony oxide skim which may be taken off and re-treated in a subsequent bath.

The process is based upon the fact that the various oxides composing the above mentioned skims may be reduced by a suitable reducing agent with the formation of either a lower oxide or the metal itself. The reducing conditions are maintained such that a part or most of the lead or antimony which may be present in the tin skim is reduced to the metallic state and again enters the bath, leaving the tin oxide in a more concentrated condition and forming substantially the entire skim. This action is further made use of in reducing the quantity of antimony skim by causing lower oxides of antimony to be formed which are readily volatilized and removed as fume, or by reducing the oxides to the metallic form.

The invention provides for greatly in-

creasing the efficiency of antimony lead separation by treating the material under alternately oxidizing and reducing conditions in order to volatilize a greater percentage of the antimony with less production of skims than has heretofore been mechanically practical.

The invention further consists in the new and novel features of operation and the new and original arrangements and combinations of steps in the process hereinafter described and more particularly set forth in the claims.

Although the novel features which are believed to be characteristic of this invention will be particularly pointed out in the claims appended hereto, the invention itself, as to its objects and advantages, the mode of its operation and the manner of its organization may be better understood by referring to the following description in which a particular commercial embodiment thereof is disclosed. It will be understood however, that the processes and the steps thereof may be modified in various respects without departing from the broad spirit and scope of the invention.

In the following description and in the claims the various steps in the process and the details comprising the invention will be identified by specific names for convenience but they are intended to be as generic in their application as the art will permit.

The process in accordance with the present invention may be carried out by heating lead bullion or alloy containing antimony and tin with or without various other impurities such as copper, arsenic, bismuth, gold and silver to a sufficiently high temperature to melt the bullion and maintaining an oxidizing atmosphere, whereby tin is oxidized and forms a skim. A suitable reducing agent is then added to the skim whereby the oxides of antimony and lead which may be enmeshed with the tin skim are reduced to the metallic state and re-enter the bath.

The skim which is considerably reduced in quantity by this means may then be removed and the process continued by raising the bullion to a suitable heat in an oxidizing atmosphere for the oxidation of the antimony, a portion of which will be passed off as a fume and may be recovered by suitable means, and another portion of which forms a skim composed essentially of lead antimony oxides on the surface of the bath. The skim is then sub-

jected to a reducing condition until greater portion of the antimony oxides have been reduced to a volatile form which passes off as a fume. The treatment is then continued, preferably by alternating the reducing and oxidizing steps until the antimony content has been reduced to the desired value. The final skim which will be comparatively small may then be removed and returned to a subsequent bath for further treatment.

As a more specific example, the process may be carried on by melting lead bullion or alloy containing, for example, 20 percent of antimony and 5 percent of tin together with smaller percentages of various other impurities such as copper, arsenic, bismuth, gold and silver, and raising the temperature very rapidly to a bright red heat while maintaining an oxidizing atmosphere. The temperature may range from 1200 to 1800 degrees F. depending upon the composition of the particular bath. Tin skims are then formed due to the oxidizing of the tin, which are reduced by submitting the bath to suitable reducing conditions as by adding fine coke having a low ash content. Since it is difficult to reduce the tin in the skims or very easy to reoxidize it while lead and, to a lesser degree, antimony are quite easy to reduce or more difficult to reoxidize this reduction treatment concentrates the tin without reducing any appreciable amount to metal.

After removal of part or all of the tin, antimony volatilizes or fumes rapidly and a skim of lead and antimony oxides appears. Whenever this skim becomes sufficiently great or for any reason appears to hinder the free oxidation and volatilization of antimony it is submitted to a reducing or partially reducing treatment as by addition of fine coke, whereby much of the antimony oxides is reduced to the volatile antimony trioxide and escapes as fume and most of the lead with some antimony is reduced to metal.

As the operation is continued and the metal bath becomes impoverished in antimony there is a greater tendency for antimony to be absorbed by the bath when a skim is reduced, hence there is an economic limit beyond which the reduction treatment of the antimony skims is not profitable. The remainder of the antimony is then removed, mainly in skims which may subsequently be reduced with a new charge of antimony-lead bearing material. By this improvement in operation the amount of antimony withdrawn from the furnace in skims and which would require retreatment to effect a separation of the antimony and lead contained therein has been greatly reduced in actual practice.

The reactions which take place during the oxidation of metals in the bath and during the reduction of the slag or skim formed during the fuming operation are complex and

vary greatly in importance according to the concentrations of the metals present and with furnace conditions. In what follows the course of the chief reactions will be described as they appear to occur according to present knowledge.

During the oxidation operation both antimony and lead are oxidized by air-oxygen but not in direct proportion to the quantities of each present since antimony is oxidized much more readily than lead at the temperature existing in the furnace. Part of the antimony trioxide thus formed escapes as fume, part is readily oxidized still further by air to the pentoxide or to the comparatively stable tetroxide, and part remains as such with the higher oxides and litharge as a slag or skim covering the metal bath. Although much of the litharge and oxides of antimony in the slag may be combined as lead antimonate when cooled, the slag may be considered as being a molten mixture of separate oxides of antimony and lead as it exists in the furnaces under the usual operating conditions. This skim or slag is beneficial when fluid and present in not too great a quantity as it serves as a medium for the further oxidation of antimony and largely prevents the volatilization of lead.

The higher oxides of antimony present in the slag near the metal bath react with the metallic antimony to produce antimony trioxide, and part of the trioxide near the surface of the slag is oxidized by air to the higher oxides. Hence there occurs in effect a transfer of air oxygen through the slag to the metallic antimony. Lead oxide, which is present in the slag, also reacts to oxidize metallic antimony and even to oxidize antimony trioxide to the higher oxides. The concentration of antimony in the bath and of each constituent in the slag as well as other factors depending upon the operating conditions present, determine to what extent and with what rapidity each of the aforementioned reactions will go.

In order to increase the rate of fuming of antimony, the atmosphere in the furnace is kept very oxidizing. This tends to rapidly oxidize antimony trioxide in the slag to the higher oxides of antimony. Unless the concentration of antimony in the metal bath is relatively high, these higher oxides are not rapidly reduced but accumulate causing a dry skim which further impedes the rapidity of their reaction with the metallic bath. By partially reducing this skim, as by application of a small amount of fine petroleum coke, the higher oxides of antimony are reduced largely to the trioxide, part of which sublimes and part remains in the slag. This results in a much smaller and a fluid slag thus greatly accelerating the volatilization of antimony. This reduction treatment also reduces lead oxide in the slag, whether free or combined

with oxides of antimony in the form of lead antimonate.

For this reduction fine low ash coke such as petroleum or pitch coke is preferred as it does not make the reduction too intense locally which would tend to put antimony back into the metal bath, nor form an objectionable slag which would interfere with the operation.

10 Arsenic, if present in the antimonial lead bath, reacts essentially as does antimony, that is, part of the arsenic present in the skim or slag is volatilized and part reduced to metal by the reducing treatment. Since the 15 percentage of arsenic present is generally very small, a relatively greater amount is reduced to metal and rejoins the metal bath than is the case with antimony.

The temperature of the metal bath during 20 the lead-antimony separation as described may range from 1200 to 1800 degrees F. and may either be held constant at some fixed temperature or intermittently be raised and lowered.

25 By reducing the quantity of skim the re-treatment necessary to recover and separate the metals contained therein is simplified and the expense and delay in removing the skims are minimized. In carrying on the process 30 the character of the conditions in the furnace may be made strongly oxidizing for the oxidation and fuming of antimony, and then changed to reducing in order to treat the skims or slag which may form in the manner above described. Not only is the amount 35 of skim which must be removed from the bath considerably reduced but the rate of volatilization of the antimony is increased.

The concentration of the tin skim by removing lead and antimony therefrom simplifies the subsequent treatment for the removal of these elements and considerably reduces the quantity of material handled.

Although certain novel features of the invention have been shown and described and are pointed out in the annexed claims, it will be understood that various omissions, substitutions and changes in the several steps of the process and in its operation may be made by those skilled in the art without departing from the spirit of the invention.

What is claimed is:

1. The process of recovering antimony from lead containing said antimony in comparatively large percentages which comprises rapidly heating said lead to a comparatively high temperature and alternately subjecting the bath to oxidizing and reducing conditions whereby volatile oxides of antimony are formed and passed off as a fume, and whereby non-volatile oxides which form a skim on the surface of the bullion are reduced to a volatile state.

2. The process of treating lead bullion containing antimony, tin and other impurities

which comprises rapidly heating said bullion to a high temperature whereby a tin skim is formed thereon, subjecting said skim to reducing conditions whereby antimony and lead oxides contained therein are partially 70 reduced to the metallic state and re-enter the bath, removing said skim and recovering tin therefrom.

3. The process of treating lead bullion containing antimony, tin and other impurities 75 which comprises rapidly heating said bullion to a temperature of from 1200 to 1800 degrees F. whereby tin skim is formed thereon, subjecting said skim to reducing conditions whereby antimony and lead oxides contained 80 therein are reduced to the metallic state and re-enter the bath, removing said skim and recovering tin therefrom.

4. The process of treating lead bullion containing antimony, tin and other impurities 85 which comprises rapidly heating said bullion to a high temperature whereby tin skim is formed thereon, adding finely divided coke to said skim whereby antimony and lead oxides contained therein are reduced to the metallic 90 state and re-enter the bath, removing said skim and recovering tin therefrom.

5. The process of treating lead bullion which comprises rapidly heating said bullion to a temperature above red heat whereby a tin 95 skim is formed thereon, subjecting said skim to reducing conditions whereby lead and antimony contained therein are reduced to a metallic state and returned to the bath, removing the concentrated skim, continuing the application of heat under oxidizing conditions 100 whereby volatile oxides of antimony are formed and whereby a smaller proportion of non-volatile oxides are formed and produce a skim, subjecting the skim to reducing conditions whereby the non-volatile oxides 105 are reduced to volatile oxides, and recovering the volatile oxides as fume.

6. The process of treating lead bullion which comprises rapidly heating said bullion 110 to a temperature above red heat whereby a tin skim is formed thereon, subjecting said skim to reducing conditions whereby lead and antimony contained therein are reduced to a metallic state and returned to the bath, 115 removing the concentrated skim, continuing the application of heat under oxidizing conditions whereby volatile oxides of antimony are formed and whereby a smaller proportion of non-volatile oxides 120 are formed and produce a skim, subjecting the skim to reducing conditions whereby the non-volatile oxides are reduced to volatile oxides, recovering the volatile oxides as fume, removing the final skim from the bath 125 and adding the same to additional quantities of lead bullion for further treatment.

7. The process of treating lead bullion which comprises rapidly heating said bullion to a temperature above red heat whereby a 130

tin skim is formed thereon, subjecting said skim to reducing conditions whereby lead and antimony contained therein are reduced to a metallic state and returned to the bath, 5 removing the concentrated skim, continuing the application of heat under oxidizing conditions whereby volatile oxides of antimony are formed and whereby a smaller proportion of non-volatile oxides are formed and produce a skim, subjecting the skim to reducing conditions whereby the non-volatile oxides are reduced to volatile oxides, recovering volatile oxides as fume, and continuing the treatment under alternately oxidizing and 10 reducing conditions until substantially all of the antimony has been removed as a fume.

8. The process of treating lead bullion which comprises rapidly heating said bullion to a temperature above red heat whereby a 20 tin skim is formed thereon, subjecting said skim to reducing conditions whereby lead and antimony contained therein are reduced to a metallic state and returned to the bath, removing the concentrated skim, continuing the application of heat under oxidizing conditions whereby volatile oxides of antimony are formed and whereby a smaller proportion of non-volatile oxides are formed and produce a skim, subjecting the skim to reducing conditions whereby the non-volatile oxides are reduced to volatile oxides, removing volatile oxides as fume, continuing the treatment under alternately oxidizing and reducing conditions until substantially all 30 of the antimony has been removed as a fume, removing the final quantity of remaining skim, and adding the same to additional amounts of lead bullion for further treatment.

40 9. The process of removing antimony from lead bullion containing antimony in comparatively large percentages, which comprises heating said bullion to a temperature above red heat, whereby a portion of the antimony is converted to a volatile oxide and removed as a fume, and further quantities of antimony are converted into non-volatile oxides which form a skim, adding a reducing agent to the bullion whereby the antimony oxide 45 skim is largely reduced to a volatile oxide of antimony, and again subjecting the bullion to oxidizing conditions for the formation of further fume.

10. The process of removing antimony from lead bullion containing antimony in 50 comparatively large percentages, which com-

prises heating said bullion to a temperature above red heat, whereby a portion of the antimony is converted to a volatile oxide and removed as a fume, and further quantities of 60 antimony are converted into non-volatile oxides which form a skim, adding finely divided coke to the bullion whereby the antimony oxide skim is largely reduced to a volatile oxide of antimony, and again subjecting the bullion to oxidizing conditions for 65 the formation of further fume.

11. The process of recovering tin and antimony from lead bullion, which comprises rapidly heating said bullion to a temperature 70 above red heat whereby a tin skim is formed, adding powdered coke to said bullion for reducing various oxides contained in said skim and concentrating the tin content thereof, removing said skim, further heating said 75 bullion under oxidizing conditions for the production of volatile and non-volatile antimony oxides, adding finely divided coke to said bullion for reducing the non-volatile oxides to volatile oxides, and further subjecting the bullion to oxidizing conditions for 80 the formation of additional quantities of volatile oxides.

12. The method of recovering antimony from lead bullion, which comprises alternately 85 subjecting said bullion to oxidizing and reducing conditions whereby lower oxides of antimony are formed and recovered as a fume.

13. The process of treating lead bullion which comprises subjecting the bullion to 90 oxidizing conditions for the formation of a tin skim, subjecting said skim to reducing conditions, and further treating said bullion in alternately oxidizing and reducing conditions whereby volatile and non-volatile oxides 95 of antimony are formed and non-volatile oxides are reduced to volatile oxides.

14. The process of treating lead bullion which comprises subjecting the bullion to 100 oxidizing conditions for the formation of a tin skim, subjecting said skim to reducing conditions for the concentration of the tin content thereof, further treating said bullion in alternately oxidizing and reducing conditions whereby volatile and non-volatile 105 oxides of antimony are formed and non-volatile oxides are reduced to volatile oxides, and recovering the volatile oxides as a fume.

In testimony whereof we have hereunto set our hands.

BRUCE WINFRED GONSER.  
CALVIN W. HAFFEY.